

Sept. 23, 1969

P. H. STEWART

3,468,664

HEAT PROCESSABLE PHOTOGRAPHIC ELEMENTS HAVING WATER  
VAPOR-IMPERMEABLE PROTECTIVE OUTER LAYER

Filed Feb. 20, 1962

EXPOSURE

Stage 1



HEATING

Stage 2

13 SILVER IMAGE



PAUL H. STEWART  
INVENTOR

BY *R. Frank Smith*

*A.H.M. Jewell*

ATTORNEY & AGENT

1

3,468,664

## HEAT PROCESSABLE PHOTOGRAPHIC ELEMENTS HAVING WATER VAPOR-IMPERMEABLE PROTECTIVE OUTER LAYER

Paul H. Stewart, Rochester, N.Y., assignor to Eastman Kodak Company, Rochester, N.Y., a corporation of New Jersey

Filed Feb. 20, 1962, Ser. No. 174,472

Int. Cl. G03c 5/30, 1/48

U.S. Cl. 96—63

19 Claims

### ABSTRACT OF THE DISCLOSURE

Photographic elements containing a developing composition and having a flexible transparent layer substantially impermeable to water vapor adhered to the outer surface of the emulsion layer, methods for processing the same, and more particularly to such photographic elements adapted to processing with heat in a relatively dry atmosphere.

This invention relates to photographic elements containing silver halide developing agents, methods for processing the same, and more particularly, to such photographic elements adapted to processing with heat in a relatively dry atmosphere.

A common procedure in the photographic art involves exposure of a silver halide emulsion layer to a subject followed by development of the resultant latent image with an alkaline solution of a silver halide developing agent such as hydroquinone to produce a silver image in the regions of the latent image. Fixing and washing steps customarily follow.

It has also been proposed to incorporate the silver halide developing agent into the sensitive element, for example, into the silver halide emulsion layer, in which case development of the exposed emulsion can be initiated merely by application of an alkaline solution. It is also known that in case both the developing agent and the alkali required to activate the developing agent are present in the sensitive element, development of the emulsion can be initiated by merely applying water.

In the Stewart et al. U.S. patent application Ser. No. 134,014 filed Aug. 5, 1961, is described a photographic process in which a sensitive element, including a silver halide emulsion layer containing a latent image, contiguous silver halide developing agent and alkali, is processed without the use of aqueous or liquid compositions by merely heating the element under relatively dry conditions thereby developing silver images in the emulsion layer.

The sensitive elements used in the Stewart et al. invention included the combination of at least one silver halide emulsion layer, a 3-pyrazolidone silver halide developing agent and an alkaline substance effective to accelerate development of a latent image in the silver halide emulsion in the presence of the developing agent. The element further included a saccharide, particularly a non-reducing oligosaccharide, such as sucrose or raffinose; and preferably, as an auxiliary developing agent, an ascorbic acid or polyhydric phenol silver halide developing agent. Additional ingredients which could be present in the sensitive element were developer preservatives such as sulfite and fog reducers such as mercaptotetrazoles or benzotriazoles. The mentioned alkaline substance, developing agent and saccharide were disposed integral with the sensitive element and contiguous to the silver halide, that is, either directly in the silver halide emulsion or in an effectively adjacent colloid layer or layers. Thus the primary developing agent, the 3-pyrazolidone compound,

2

could be present in the silver halide emulsion and the auxiliary developing agent, alkali and saccharide in an adjacent colloid layer. Similarly, both developing agents, alkali and saccharide, could be present in a layer underlying or overlying the emulsion on a support. Useful combinations of developer ingredients, included a 3-pyrazolidone developing agent as the sole developing agent, in combination with a saccharide; a 3-pyrazolidone in combination with an ascorbic acid and, if desired, a saccharide, and the combination of a 3-pyrazolidone developing agent, a polyhydric phenol developing agent, and if desired, a saccharide.

The process of the Stewart et al. invention further embodied the steps of recording latent images in the 15 silver halide emulsions in the presence of the developing agents and other ingredients mentioned above, followed by heating the emulsion sufficiently to develop silver images therein. In a representative procedure, the sensitive element containing the mentioned ingredients and a small 20 amount of moisture was exposed to a subject, then subjected to heat by passing over a heated roller at temperatures of the order of 50 to 200° C. As a result a silver image was developed in the emulsion layer. In another procedure, an exposed sensitive element containing the 25 mentioned ingredients was passed at speeds of the order of 10 to 200 feet per minute through a heated chamber so designed that moisture rising from heating of the sensitive element was confined within the chamber and a combination of heat and moisture thus obtained initiated 30 development. The exposed sensitive elements could also be processed by subjecting them to the action of hot air, containing a moderate amount of moisture. Moist steam could be used but it was not required. One disadvantage of that process was that the print could not be 35 viewed as it was developed because the apparatus including the processing chamber obscured the print. If the top of the chamber was removed to afford view of the print during processing, moisture escaped and image quality was greatly reduced.

I have discovered that the sensitive elements described above which contain silver halide and contiguous developing agent and alkali can be viewed while being processed and still produce prints having good photographic quality 45 if the outer surface of the silver halide emulsion layer is provided with a flexible transparent coating resistant to the penetration of water vapor. That is, as mentioned above, the development process requires that a small amount of moisture be present in the sensitive element together with the silver halide developing agent and alkali, in order that the development of the exposed silver 50 halide will proceed upon application of heat. In the Stewart et al. invention it was preferred for best results to confine the moisture to the sensitive element in some manner such as by use of special processing equipment 55 designed to confine the moisture near the surface of the emulsion layer.

According to my invention, when the transparent coating 60 is applied to the surface of the emulsion layer, which coating is resistant to moisture penetration and preferably is substantially impervious to moisture vapor, upon heating the exposed emulsion layer moisture is effectively trapped in the element and development quickly 65 proceeds with the result that prints of good quality are obtained. Thus, the equipment used for heating the sensitive element over a heated surface preferably with the emulsion support in contact therewith with the result that development quickly proceeds and the print can be viewed immediately thereafter.

While useful results can be obtained with other silver 70 halide developing agents having high development activity, the 3-pyrazolidone developing agents are preferred

components of the sensitive elements and are unique in their activity in the dry development process of the invention as compared to other silver halide developing agents. Thus, when one sensitive element containing both 1-phenyl-3-pyrazolidone and ascorbic acid and a second element containing both monomethyl-p-aminophenol and hydroquinone are exposed and heated under various conditions, a low density silver image is obtained in the latter element. On the other hand, the 3-pyrazolidone-ascorbic acid system of the invention yields a high density silver image under the same conditions of treatment.

Moreover, it is important that a substantial amount of the 3-pyrazolidone developing agent in addition to the alkali be present in the silver halide emulsion or in a contiguous layer. For example, an emulsion containing no alkali and no more than about two grams of 3-pyrazolidone compound per mole of silver halide, upon exposure and heating yields no visible silver image. When about 10 to 50 grams of 3-pyrazolidone compound per mole of silver halide is present, only a faint visible image is obtained upon heating in the absence of alkali. However in the presence of alkali, about 15 to 25 grams of 3-pyrazolidone per mole of silver halide is sufficient to produce a high density silver image upon heating the latent image. When an auxiliary developing agent such as ascorbic acid or hydroquinone is present in addition to the 3-pyrazolidone compound and a saccharide, as little as five grams of 3-pyrazolidone developing agent per mole of silver halide is sufficient. Of course, if desired, the 3-pyrazolidone-containing emulsions free of alkali may be developed with alkaline solutions containing additional developing agents as Elon and hydroquinone.

The accompanying drawing shows in greatly enlarged cross-sectional view the appearance of a representative sensitive element of the invention at different stages of processing. Equipment particularly useful for heating the sensitive element of the invention is described in the Stewart U.S. patent application Ser. No. 147,899 filed Oct. 26, 1961 comprising a grooved heated element over which the exposed sensitive element is passed with the emulsion support in contact with the heated surface.

In the element of FIG. 1 of the drawings, layer 10 represents a support such as synthetic resin or cellulose ester, preferably paper, carrying a silver halide emulsion layer 11, a 3-pyrazolidone developing agent and alkali integral and contiguous to the silver halide and, if desired, other ingredients such as the auxiliary developing agent and a saccharide. Layer 12 represents a transparent layer substantially impermeable to moisture such as a cellulose ester or synthetic polymer coating or laminate serving to confine moisture to the element during the heat development step.

As shown in Stage 1 of the drawings, the process of the invention includes the exposure of the sensitive element to a subject to record a latent image in the silver halide in area 13 of layer 11. Thereafter, the element is heated sufficiently to develop a silver image in area 13 as shown in Stage 2. In this process, it will be observed that when the sensitive element is heated, a visible silver image is obtained instantaneously. This result is facilitated by the use in the emulsion layer of silver halides which have short development induction periods, such as fine grain silver bromide emulsions. Emulsion having longer induction periods are useful but require longer application of heat to effect their development in the processes of the invention. Also it has now been found that the use of the moisture impervious layer 12 facilitates the rapid production of a visible silver image in these emulsions, the effect being especially pronounced with the emulsion possessing longer development induction periods.

The 3-pyrazolidone silver halide developing agents, such as those described below, are useful in our invention. The 3-pyrazolidone compounds having the follow-

ing general Formula I are particularly useful in the sensitive elements.



10 in which the various R groups represent substituents such as hydrogen, alkyl, acyl, heterocyclic or aryl groups, for example, R1 can be benzothiazolyl or an aryl group of the benzene or naphthalene series, substituted or not. R1, R2, R3, R4 and R5 can be hydrogen atoms or alkyl groups of from 1 to 12 carbon atoms or aryl groups such as phenyl and naphthyl, substituted or not. Typical substituents are lower alkyl groups, including haloalkyl, pyridinium- or picolinium-N-alkyl halide, e.g. pyridinium-N-methyl chloride, benzyl, phenyl, 4-methylphenyl, 4-methoxyphenyl, carboxylic acid acyl as acetyl, benzoyl, nitrobenzoyl and haloacetyl, e.g. chloroacetyl, phenoxy and alkylphenoxy.

15 The 3-pyrazolidone developing agents of our invention which are used to advantage particularly with gold and sulfur sensitized silver halide emulsions are represented by the following formulas:



40 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495

- (4) 1-phenyl-2-benzoyl-3-pyrazolidone
- (5) 1-p-chlorophenyl-3-pyrazolidone
- (6) 1-phenyl-5-phenyl-3-pyrazolidone
- (7) 1-m-tolyl-3-pyrazolidone
- (8) 1-phenyl-5-methyl-3-pyrazolidone
- (9) 1-p-tolyl-5-phenyl-3-pyrazolidone
- (10) 1-m-tolyl-3-pyrazolidone
- (11) 1-p-methoxyphenyl-3-pyrazolidone
- (12) 1-acetamidophenyl-3-pyrazolidone
- (13) 1-phenyl-2-acetyl-4,4-dimethyl-3-pyrazolidone
- (14) 1-phenyl-4,4-dimethyl-3-pyrazolidone
- (15) 1-m-aminophenyl-4-methyl-4-propyl-3-pyrazolidone
- (16) 1-o-chlorophenyl-4-methyl-4-ethyl-3-pyrazolidone
- (17) 1-m-acetamidophenyl-4,4-diethyl-3-pyrazolidone
- (18) 1-(p- $\beta$ -hydroxyethylphenyl)-4,4-dimethyl-3-pyrazolidone
- (19) 1-p-hydroxyphenyl-4,4-dimethyl-3-pyrazolidone
- (20) 1-p-methoxyphenyl-4,4-diethyl-3-pyrazolidone
- (21) 1-p-tolyl-4,4-dimethyl-3-pyrazolidone
- (22) 1-(7-hydroxy-2-naphthyl)-4-methyl-4-n-propyl-3-pyrazolidone
- (23) 1-p-diphenyl-4,4-dimethyl-3-pyrazolidone
- (24) 1-(p- $\beta$ -hydroxyethylphenyl)-3-pyrazolidone
- (25) 1-o-tolyl-3-pyrazolidone
- (26) 1-o-tolyl-4,4-dimethyl-3-pyrazolidone
- (27) 1-benzothiazolyl-3-pyrazolidone
- (28) 1-phenyl-2-p-nitrobenzoyl-3-pyrazolidone
- (29) 1-phenyl-2-carbethoxy-3-pyrazolidone
- (30) 1-phenyl-2-( $\alpha$ -2,4-di-t-amylphenoxybutyl)-3-pyrazolidone
- (31) 1-phenyl-2-phenoxyacetyl-4-methyl-3-pyrazolidone
- (32) 1-phenyl-2-lauroyl-3-pyrazolidone
- (33) 1-phenyl-2-acetyl-3-pyrazolidone
- (34) 1-phenyl-2-chloroacetyl-3-pyrazolidone
- (35) 1-phenyl-3-acetyl-4-methyl-3-pyrazolidone
- (36) 1-p-tolyl-2-acetyl-3-pyrazolidone
- (37) 1-p-chlorophenyl-2-acetyl-3-pyrazolidone



- (38) 2-(pyridinium acetyl)-1-phenyl-3-pyrazolidone chloride
- (39) 2-(pyridinium acetyl)-4-methyl-1-phenyl-3-pyrazolidone chloride
- (40) 2-(pyridinium acetyl)-4-dimethyl-1-phenyl-3-pyrazolidone chloride



- (41) Enol acetate of 1-phenyl-3-pyrazolidone



- (42) Enol acetate of 4-methyl-1-phenyl-3-pyrazolidone

Compounds 1 to 12 can be prepared by the methods described in British Patents 679,677 and 679,678. Compounds 13 to 23 and 26 above are representative of 4,4-dialkyl-3-pyrazolidone compounds useful in this invention and these compounds are described in Allen et al. U.S. Patent 2,772,282, Nov. 27, 1956.

The  $\omega$ -hydroxyalkylphenyl-3-pyrazolidones in which the alkyl group preferably contains from 1 to 4 carbon atoms, for example, compounds 18 to 24 above, are described in Allen et al. invention and in Reynolds and Tinker U.S. Patent 2,743,279, Apr. 24, 1956.

Compounds 33 to 35 and 38 to 42 may be prepared as described in U.S. Ser. No. 134,014 above mentioned.

While the processes of the invention can be carried out with sensitive elements containing a 3-pyrazolidone silver halide developing agent as the sole developing agent, in a preferred embodiment of the invention a 3-pyrazolidone developing agent is used in combination with ascorbic acid silver halide developing agent, such as d- and L-ascorbic acids, d-arabo ascorbic acid, iminogluco-ascorbic acid and other ascorbic acids having the formulas shown in James et al., U.S. Patent 2,688,549, granted Sept. 7, 1954. Alternately, the 3-pyrazolidone developing agents are employed in combination with a polyhydric phenol silver halide developing agent such as hydroquinone, catechol, 4-phenylcatechol or pyrogallol. As mentioned previously, when a 3-pyrazolidone is used in combination with these auxiliary developing agents, appreciably less of the 3-pyrazolidone compound is required in the sensitive element to maintain high development activity and thus produce the silver images with a minimum of heating of the exposed emulsion layer.

The saccharides have previously been employed in a sensitive element in order to improve the stability of the emulsion upon aging for extended periods of time. In the present invention of the saccharides, especially the non-reducing oligosaccharides, such as sucrose and raffinose, permit use of much less developing agent in the freshly coated sensitive element than would be the case if the saccharide were absent. Representative saccharides which may be used are: fructose, glucose, inulin, melezitose, pectin, raffinose, starch, sucrose and trehalose. The non-reducing oligosaccharides such as sucrose and raffinose are especially useful.

"Non-reducing" has a meaning herein usually applied to saccharides and means that the compounds are members of the class of saccharides which do not reduce alkaline solutions of salts of metals such as copper salts, as present in Fehling's solution, as compared to reducing sugars like fructose.

Useful amounts of the various ingredients in the sensitive elements can be ascertained from the following examples although optimum qualities should be ascertained by experiment under the particular conditions in use. However, 3-pyrazolidone compound such as 1-phenyl-3-pyrazolidone may be used in amounts in excess of about 20 grams per mole of silver halide and when in combination with an auxiliary developing agent such as, ascorbic acid or hydroquinone, an amount in excess of about 5 grams per mole of silver halide should be used. Quantities of the 3-pyrazolidones in excess of about 50 grams per mole of silver halide may be difficult to disperse in many silver halide emulsions. However, somewhat larger amounts of from about 50 to 300 grams per mole of silver halide can be used. The saccharides may be used in combination with the pyrazolidones in amounts ranging from about 30 to 1000 grams per mole of silver halide. If too large a quantity is used, crystallization occurs or the emulsion tends to be tacky, depending upon the particular saccharide used. The auxiliary developing agents such as the ascorbic acids may be used in combination with the 3-pyrazolidones in amounts of the order of about 30-600 grams per mole of silver halide and the polyhydric phenol developers such as hydroquinone in the range of about 15 to 75 grams per mole of silver halide.

However, at the higher levels of concentration, the latter developing agent tends to produce more background stain in the prints than desired.

The alkaline materials present in the sensitive elements together with the developing agents include inorganic alkalies such as alkali metal metaborate and carbonate. Organic alkaline materials such as quaternary ammonium bases and amines such as 2-amino-2-methyl-1,3-propane diol can be used. The inorganic alkalies which do not yield volatile bases upon heating are very useful.

As mentioned, the sensitive element should contain a small amount of moisture at the time of heating to develop the image. A useful amount of moisture is that remaining in a sensitized paper, such as prepared in Example 1, upon drying and handling at about 75° F. and 30 to 50% RH e.g., about 5 to 10% moisture.

The emulsion addenda described in the Stewart et al. U.S. patent application Ser. No. 134,014 mentioned, including the noble metal salts, stannous salts, polyamines, optical sensitizing dyes, stabilizing compounds, chemical sensitizing compounds, plasticizers, gelatin hardeners, coating aids and colloid vehicles disclosed therein may be used advantageously in the present emulsions. The silver halide emulsions may be varied considerably and include silver bromide, silver chloride, silver iodide and combinations of these such as chlorobromide, chlorobromoiodide or bromoiodide.

The coatings, which are applied to the emulsion layer to resist penetration of water vapor resulting from heating of the sensitive element, can be applied to the emulsion layer by various methods including coating aqueous or organic solvent solutions or dispersions of organic film-forming polymeric materials upon the emulsion layer or by the lamination of thin transparent polymeric sheets onto the emulsion layers. In one method a thin transparent foil such as cellulose acetate sheeting can be merely pressed into contact with the emulsion surface without using any particular adhesive and the cellulose acetate sheet adheres sufficiently to the emulsion surface to confine the moisture to the emulsion during the heating step. Thus, in those cases where the moisture impervious layer is not permanently adhered to the emulsion layer, it may be desirable following processing to detach the coating in order to allow further photographic operations such as fixing to be performed upon the developed emulsion layer. The lamination of such sheeting onto the emulsion can be performed either prior to or subsequent to exposure of the emulsion layer to the subject. In another procedure illustrated in the examples below, aqueous dispersions or latices containing synthetic polymers resistant to moisture are suitable for coating upon the emulsion layers to provide the same moisture impervious layers.

The following examples will serve to illustrate my invention.

#### EXAMPLE 1

To a gelatino silver bromoiodide emulsion which was optically sensitized was added, per mole of silver halide, 1.5 gm. 1-phenyl-5-mercaptopotetrazole, 640 gm. sucrose, 162 gm. ascorbic acid, 30 gm. 1-phenyl-3-pyrazolidone, 36 gm. sodium sulfite (anhy.) 540 gm. sodium metaborate octahydrate, and 12 gm. potassium bromide. The emulsion was coated on a paper base at a coverage of about 1500 square feet per mole silver halide. A 50% polyvinylidene chloride latex "Resyn 3600" manufactured by the National Starch Company, 750 3rd Ave., New York, N.Y., was adjusted to a pH of 9.5 with 2.5 N NaOH and coated upon the emulsion layer at a coverage of about 7.5 gm. latex per square foot.

The resulting sensitive element appears substantially as shown in Stage 1 of the drawing, the emulsion layer 11 being supplied with the flexible substantially moisture impervious polymeric layer 12 obtained by coating the polymeric latex thereon. Samples of this sensitive paper, and "Control" samples of the same paper not provided

75

with the polymeric layer, were exposed to a subject then advanced at 3 ft. per minute for a distance of about 4 inches over a curved metal surface heated to 150° C. with the result that silver images quickly became visible. After processing in this manner, the exposed element of Stage 1 appears substantially as shown in Stage 2 the emulsion layer 11 containing the silver image 13. As a result of processing both of the papers, silver images were readily visible in each emulsion layer, but the paper of the invention carrying the transparent polymeric coating 12 upon the emulsion layer had a speed 0.26 relative log E faster, at a density of 0.1 above fog, than the paper not provided with the polymeric coating.

In a similar manner, the sensitive elements comprising silver halide developing agent and alkali can be coated with latices of various types capable of yielding transparent coatings resistant to moisture penetration, depending upon the moisture repellent properties of the polymeric component of the latex. Thus, polyvinyl ester latices, such as "Flexac," a latex containing 50% polyvinyl ester manufactured by the Colton Chemical Company, have been found to be very useful in place of the latex used in Example 1.

#### EXAMPLE 2

The same ingredients were added to a gelatino silver chlorobromoiodide emulsion as in Example 1, except using 5.0 grams of 1-phenyl-5-mercaptopotetrazole, and the emulsion was coated upon a paper base at a coverage of about 1500 sq. ft. per mole of silver halide. A transparent adhesive sheet, "Scotch" Brand Cellophane Tape, manufactured by Minnesota Mining and Manufacturing Company, St. Paul, Minn., was laminated to the surface of the emulsion layer and strips of the resultant element, together with strips of the Control sample not provided with the adhesive sheet over the emulsion layer, were exposed to a subject and each strip passed over a metal surface heated to 150° C. at different speeds to develop silver images therein with the results shown in the following table:

|                                              | Paper Travel Speed (ft./min.) |      |      |      |      |
|----------------------------------------------|-------------------------------|------|------|------|------|
|                                              | 0.5                           | 1.0  | 2.0  | 3.0  | 5.0  |
| $D_{max}$ . of control strips.....           | 0.74                          | 0.76 | 0.55 | 0.48 | 0.38 |
| $D_{max}$ . of strips laminated to tape..... | 1.14                          | 1.12 | 1.06 | 1.02 | 0.70 |

From the data in the above table, it will be apparent that with varying amounts of heat represented by the different paper travel speeds, the sensitive element of the invention provided with the adhesive sheet overlying the emulsion layer yielded silver images having substantially greater density. In a similar manner, other transparent adhesive tapes such as the transparent polyester adhesive tape No. 850 sold by the Minnesota Mining and Manufacturing Company can be used in the manner of this example to apply a moisture impervious layer to the emulsion surface.

It has also been found that in processes of the above type, the rate of development may be increased and the background density of the prints improved by the incorporation of a silver halide solvent such as sodium thiosulfate into the sensitive element as follows: A gelatino silver halide emulsion containing sucrose, ascorbic acid, 1-phenyl-3-pyrazolidone, sodium sulfite, sodium metaborate, potassium bromide and sodium thiosulfate was coated on a paper (or film) base and air dried; also, a control coating with the sodium thiosulfate omitted was made. Imagewise exposed strips of both coatings were then subjected to air saturated with moisture at 95-100° C. for a time sufficient for the prints to be stable when exposed to actinic light under high relative humidity conditions. The coating containing sodium thiosulfate required a considerably shorter processing time than that required for the control, and the background density of the print was lower than that of the control print. The process can be carried out as shown in detail in the following example.

## EXAMPLE 3

A gelatino silver bromoiodide emulsion containing 640 g. sucrose, 162 g. ascorbic acid, 30 g. 1-phenyl-3-pyrazolidone, 36 g. sodium sulfite, 540 g. sodium metaborate octahydrate, 12 g. potassium bromide and 117.6 g. sodium thiosulfate pentahydrate ( $\text{Na}_2\text{S}_2\text{O}_3 \cdot 5\text{H}_2\text{O}$ ) per mole silver halide was coated on single weight paper stock at a coverage of approximately 1600 ft.<sup>2</sup> per mole silver halide, and then air dried. A control coating with the sodium thiosulfate omitted was made. An imagewise exposed strip of the coating containing sodium thiosulfate, when subjected to air saturated with water at 99° C. for 1 second, gave a legible print. The control coating required a 10" processing time, and the background density of the print was 0.18 higher than that of the print containing sodium thiosulfate. Detailed sensitometric data appear in the following table:

| $\text{Na}_2\text{S}_2\text{O}_3 \cdot 5\text{H}_2\text{O}$<br>(g./mole $\text{AgX}$ ) | Processing<br>time, <sup>1</sup><br>seconds | Relative<br>Speed | $D_{\min}$ |
|----------------------------------------------------------------------------------------|---------------------------------------------|-------------------|------------|
| 117.6                                                                                  | 1                                           | 269               | 0.29       |
| 0                                                                                      | 10                                          | 100               | 0.47       |

<sup>1</sup> Air saturated with moisture at 99° C.

The above Example 3 demonstrates that silver halide solvents, such as sodium thiosulfate, are very effective for increasing the development rate and reducing the background density of these materials.

## EXAMPLE 4

A gelatino-silver bromoiodide emulsion containing 640 g. sucrose, 162 g. ascorbic acid, 30 g. 1-phenyl-3-pyrazolidone, 36 g. sodium sulfite, 540 g. sodium metaborate octahydrate, 12 g. potassium bromide, 157 g. sodium thiosulfate pentahydrate ( $\text{Na}_2\text{S}_2\text{O}_3 \cdot 5\text{H}_2\text{O}$ ) and 10 g. 1-phenyl-5-mercaptopentetrazole per mole of silver was coated on single weight paper stock at a coverage of approximately 1600 sq. ft. per mole of silver halide and then air dried. A 35 mm. wide control strip of the above coating was given an imagewise exposure and then processed at a paper travel speed of  $\frac{1}{2}$  ft. per min. by means of the processor described in the Stewart U.S. patent application Ser. No. 147,899 filed Oct. 6, 1961 (an apparatus including a convexly curved heated metal surface containing a plurality of transverse grooves adapted to trap moisture driven out of paper passed over the surface) operating at a temperature of 150° C. The coated side of a similar strip, after imagewise exposure, was laminated to an adhesive tape similar to that described in Example 2 and processed in a similar manner. The following data were obtained.

|                               | Relative<br>speed | Contrast | $D_{\max}$ |
|-------------------------------|-------------------|----------|------------|
| Control                       | 100               | 0.1      | 0.5        |
| Coated side laminated to tape | 2,190             | 0.3      | 0.8        |

Samples similar to those described above were also, after an imagewise exposure, processed at the paper speeds listed below in an apparatus similar to the one described above in this example but which was additionally equipped with a moisture-saturated wick extending from a reservoir of water into a steam chamber operating at a temperature of 105° C. to convert the water in the wick to steam. This steam can be conducted to the transverse grooves in the convexly curved heated metal surface by means of perforations extending through the metal surface from the steam chamber which may be at the back of said metal surface. Or the heated metal surface could be formed from a block of one of the commercially available sintered porous metals to overcome the problem of perforating the metal block to permit transfer of the

steam from the back surface to the convexly curved surface of the same. The following data apply.

|                                                               | Relative<br>speed | Contrast | $D_{\max}$ |
|---------------------------------------------------------------|-------------------|----------|------------|
| Control (paper travel speed $\frac{1}{2}$ ft./min.)           | 795               | 0.1      | 0.6        |
| Coated side laminated to tape (paper travel speed 1 ft./min.) | 4,470             | 0.4      | 1.0        |

The invention has been described in considerable detail with particular reference to preferred embodiments thereof, but it will be understood that variations and modifications can be effected within the spirit and scope of the invention as described hereinabove and as defined in the appended claims.

What I claim is:

1. A non-light exposed light-sensitive element containing a small amount of moisture and comprising a support having thereon a silver halide emulsion layer, a silver halide developing agent and an alkaline material being integral with and contiguous to the silver halide and an integral flexible transparent layer resistant to penetration by water vapor as an outermost layer to seal said moisture in said element.
2. The element of claim 1 wherein the developing agent is present in the emulsion layer and the alkali in a layer separate from the emulsion layer.
3. The element of claim 1 wherein the developing agent is present in the emulsion layer and the alkali in a layer overlying the emulsion layer.
4. A light-sensitive element of claim 1 in which the support is paper.
5. A non-light-exposed light-sensitive element containing a small amount of moisture and comprising a paper support having thereon a silver halide emulsion layer, at least about 5 gms. per mole silver halide of a 3-pyrazolidone silver halide developing agent, a non-reducing saccharide and an alkaline material being integral with and contiguous to the silver halide, and an integral flexible transparent layer resistant to penetration by water vapor adhered to the outer surface of the emulsion layer.
6. A non-light-exposed light-sensitive element containing a small amount of moisture and comprising a paper support having thereon a silver halide emulsion layer, at least about 15 gms. per mole of silver halide of a silver halide developing agent of the class consisting of polyhydric phenol and ascorbic acid developing agents, at least about 5 gms. per mole silver halide of a 3-pyrazolidone silver halide developing agent and an alkaline material being integral with and contiguous to the silver halide, and an integral flexible transparent layer resistant to penetration by water vapor adhered to the outer surface of the emulsion layer.
7. A non-light exposed light-sensitive element containing a small amount of moisture and comprising a paper support having thereon a silver halide emulsion layer, at least about 15 gms. per mole silver halide of a polyhydric phenol developing agent, at least about 5 gms. per mole silver halide of a 3-pyrazolidone silver halide developing agent and an alkaline material being integral with and contiguous to the silver halide, and an integral flexible transparent layer resistant to penetration by water vapor adhered to the outer surface of the emulsion layer.
8. A non-light exposed light-sensitive element containing a small amount of moisture and comprising a paper support having thereon a silver halide emulsion layer, at least about 15 gms. per mole silver halide of ascorbic acid, at least about 5 gms. per mole silver halide of a 3-pyrazolidone silver halide developing agent and an alkaline material being integral with and contiguous to the silver halide and an integral flexible transparent layer resistant to penetration by water vapor adhered to the outer surface of the emulsion layer.
9. The element of claim 3 further containing ascorbic acid integral with and contiguous to the silver halide.

10. The element of claim 1 wherein the alkaline material is an alkali metal metaborate.

11. A photographic process comprising exposing to a subject a light-sensitive photographic element containing water, including a support having thereon a photosensitive emulsion layer, a developing composition for said photosensitive emulsion layer, and a flexible transparent layer substantially impermeable to water vapor adhered to the outer surface of the emulsion layer, and heating said element whereby said water activates the developer composition until an image is obtained in the emulsion layer.

12. A photographic process comprising exposing to a subject a light-sensitive photographic element containing water, including a support having thereon a silver halide emulsion layer, a silver halide developing composition, and a flexible transparent layer substantially impermeable to water vapor adhered to the outer surface of the emulsion layer, and heating said element whereby said water activates the developer composition until a silver image is obtained in the emulsion layer.

13. A photographic process comprising exposing to a subject a light-sensitive photographic element including a support having thereon a silver halide emulsion layer, a halide developing agent and an alkaline material being integral with and contiguous to the silver halide and an integral flexible transparent layer substantially impermeable to water vapor adhered to the outer surface of the emulsion layer, and heating said element containing a small amount of moisture until a silver image is obtained in the emulsion layer.

14. A photographic process which comprises exposing to a subject a light-sensitive element containing a small amount of moisture and comprising a paper support having thereon a silver halide emulsion layer, a 3-pyrazolidone silver halide developing agent and an alkaline material being integral with and contiguous to the silver halide, and an integral flexible transparent layer resistant to penetration by water vapor adhered to the outer surface of the emulsion layer, and heating said element until a silver image is obtained in the emulsion layer.

15. A photographic process which comprises exposing to a subject a light-sensitive element containing a small amount of moisture and comprising a paper support having thereon a silver halide emulsion layer, at least about 5 gms. per mole silver halide of a 3-pyrazolidone silver halide developing agent, a non-reducing saccharide and an alkaline material being integral with and contiguous to the silver halide, and an integral flexible transparent layer resistant to penetration by water vapor adhered to the outer surface of the emulsion layer, and heating said element until a silver image is obtained in the emulsion layer.

16. A photographic process which comprises exposing to a subject a light-sensitive element containing a small amount of moisture and comprising a paper support having thereon a silver halide emulsion layer, at least about 15 gms. per mole of silver halide of a silver halide developing agent of the class consisting of polyhydric phenol and ascorbic acid developing agents, at least about 5 gms. per mole silver halide of 3-pyrazolidone silver halide developing agent and an alkaline material being integral with and contiguous to the silver halide, and an integral flexible transparent layer resistant to penetration by water vapor adhered to the outer surface of the emulsion layer, and heating said element until a silver image is obtained in the emulsion layer.

17. A photographic process which comprises exposing to a subject a light-sensitive element containing a small amount of moisture and comprising a paper support having thereon a silver halide emulsion layer, at least about 15 gms. per mole silver halide of a polyhydric phenol developing agent, at least about 5 gms. per mole silver halide of a 3-pyrazolidone silver halide developing agent and an alkaline material being integral with and contiguous to the silver halide, and an integral flexible transparent layer resist to penetration by water vapor adhered to the outer surface of the emulsion layer, and heating said element until a silver image is obtained in the emulsion layer.

18. A photographic process which comprises exposing to a subject a light-sensitive element containing a small amount of moisture and comprising a paper support having thereon a silver halide emulsion layer, at least about 15 gms. per mole silver halide of ascorbic acid, at least about 5 gms. per mole silver halide of a 3-pyrazolidone silver halide developing agent and an alkaline material being integral with and contiguous to the silver halide and an integral flexible transparent layer resistant to penetration by water vapor adhered to the outer surface of the emulsion layer, and heating said element until a silver image is obtained in the emulsion layer.

19. The process of claim 11 wherein the element further contains ascorbic acid integral with and contiguous to the silver halide.

#### References Cited

##### UNITED STATES PATENTS

3,248,219 4/1966 Jacobs \_\_\_\_\_ 96—76

NORMAN G. TORCHIN, Primary Examiner

C. E. DAVIS, Assistant Examiner

U.S. Cl. X.R.

96—48, 50, 76, 95

UNITED STATES PATENT OFFICE  
CERTIFICATE OF CORRECTION

Patent No. 3,468,664 Dated 9/23/69

Inventor(s) Paul H. Stewart

It is certified that error appears in the above-identified patent and that said Letters Patent are hereby corrected as shown below:

Col. 10, line 50, between "with" and "contiguous", delete "an" and substitute in its place --and--; line 52, between "to" and "by", delete "penertation" and substitute in its place --penetration--; line 62, between "to" and "by", delete "penertation" and substitute in its place --penetration--.

Col. 11, lines 24/25, between "emulsion layer, a" and "halide developing", add --silver--.

Col. 12, line 2, between "light-" and "element", delete "sensitieve" and substitute in its place --sensitive--; line 24 between "layer" and "to", delete "resist" and substitute in its place --resistant--.

SIGNED AND  
SEALED  
JAN 19 1971

(SEAL)

Attest:

Edward M. Fletcher, Jr.

Attesting Officer

WILLIAM E. SCHUYLER, JR.  
Commissioner of Patents